

## UNITED STATES PATENT OFFICE

GEORGE P. HALLIWELL, OF WILKINSBURG, PENNSYLVANIA, ASSIGNOR TO WESTINGHOUSE ELECTRIC & MANUFACTURING COMPANY, A CORPORATION OF PENNSYLVANIA

## THERMIONIC CATHODE

No Drawing.

Application filed December 14, 1928. Serial No. 326,155.

My invention relates to thermionic tubes or space discharge devices and more particularly to an improved thermionic cathode for such devices that is capable of emitting 5 electrons.

An object of my invention is to provide an inexpensive cathode for space discharge devices, such as thermionic tubes, that has uniform physical properties and which is 10 capable of emitting electrons at temperatures lower than cathodes composed of oxide-coated platinum or platinum alloys.

Another object of my invention is to provide an improved alloy or aggregate for the 15 cathodes of space discharge devices that has a comparatively high specific resistance, that may be made from cheap and readily obtainable materials and that has physical properties which are superior to oxide-coated 20 filaments.

Another object of my invention is to provide improved vacuum tubes or space discharge devices, and especially those of the three or four electrode type having output 25 and control electrodes, and a cathode comprising an alloy or aggregate that is capable of emitting electrons when heated to a moderately high temperature.

A further object of my invention is to provide a method of producing an alloy or aggregate in which one or more of the alkaline 30 earth metal oxides are incorporated that may be forged and drawn into wires or filaments capable of being utilized as the cathode in 35 space discharge devices.

It has heretofore been the practice to employ tungsten, thoriated tungsten and oxide-coated filaments of platinum or platinum alloys as the cathode in space discharge 40 devices, such as X-ray tubes, hot cathode rectifiers and vacuum tubes of the three and four electrode type that are utilized for radio purposes.

Vacuum tubes having cathodes made of 45 tungsten or thoriated tungsten have a comparatively short life and the electron emission is somewhat irregular. Oxide coated filaments having a foundation metal of platinum or nickel, or alloys of these metals, have 50 been in extensive use. Oxide coated fila-

ments, however, are not altogether satisfactory because of the difficulty of producing filaments of this type having uniform physical properties.

In producing oxide coated cathodes in accordance with the present practice, it is difficult to obtain a filament having an adherent layer of the oxide or one which has a uniform thickness of the oxide coating on the wire. There is also considerable difficulty 55 in obtaining true temperature measurements of oxide-coated filaments to determine the temperature at which the tube is to be operated because they are formed of two layers; namely, the foundation metal and the 60 superimposed oxide coating. Oxide-coated filaments also have a rough soft surface and care must, therefore, be exercised in handling the material to prevent the oxide coating from being removed or contaminated 65 with oil or grease while it is being mounted 70 in the tube.

The mechanism of thermionic emission from oxide coated surfaces is not clearly 75 understood, but according to the latest theory, part of the oxide is reduced to the metallic state in minute quantities which forms a superficial filament of high thermionic activity. Only a layer of metal one molecule 80 thick is presumed to give satisfactory emission.

In making experiments in accordance with the above specified theory, I have made the discovery that when an alkaline-earth-metal oxide is disseminated through or alloyed 85 with a metal which is suitable as a base for electron emitting bodies, such as nickel, to which is added a metal which is highly active toward oxygen, such as titanium, a filament material is provided that not only gives good 90 emission, but is free from the disadvantages resulting from the use of oxide-coated material.

In practicing my invention, I may form 95 intimately powdered mixtures of a foundation metal, such as nickel with a metal which is highly active toward oxygen, such as titanium, and the oxides of one or more of the alkaline earth metals, such as calcium, 100 barium or strontium, or I may mix pow-

1,888,888  
+ of

such a composition have good physical properties and also have the advantage of giving electron emission at about 100° C. lower temperature than platinum. A small percentage of other metals which are highly active toward oxygen, such as thorium, vanadium, tantalum, silicon, manganese, aluminum, or metals of the rare earth group such as cerium or zirconium, or mixtures thereof, may be 10 substituted in whole or in part for the titanium.

Other modifications of my invention will become apparent to those skilled in the art, and I desire, therefore, that only such limitations shall be placed on my invention as are imposed by the prior art and the appended 18 claims.

I claim as my invention:

1. Electron emitting material of substantially homogeneous character capable of being forged into wire consisting of a base metal selected from a group consisting of nickel and cobalt, said base metal containing about 0.5 per cent titanium and about 10 per cent metal selected from a group consisting of titanium and iron, with about 2 to 10 per cent alkali-earth metal oxide uniformly distributed therethrough.

2. Electron emitting material of substantially homogeneous character capable of being forged into wire consisting of a base metal of about 70 per cent nickel, 20 per cent cobalt, 0.5 per cent titanium and the balance selected from a group consisting of iron and titanium, with about 2 to 10 per cent alkali-earth metal oxide uniformly disseminated therethrough.

3. Electron emitting material of substantially homogeneous character capable of being forged into wire consisting of a base metal of about 70 per cent nickel, 20 per cent cobalt, 8 per cent iron and 2 per cent titanium with about 4 per cent alkali-earth metal oxide uniformly distributed therethrough.

45 In testimony whereof, I have hereunto subscribed my name this 12th day of December 1928.

GEORGE P. HALLIWELL.